

## UNITED STATES PATENT OFFICE.

KURT H. MEYER AND HERMANN SCHÜTTE, OF MANNHEIM, GERMANY, ASSIGNEES TO  
I. G. FARBENINDUSTRIE AKTIENGESELLSCHAFT, OF FRANKFORT-ON-THE-MAIN,  
GERMANY.

## PROCESS OF TANNING HIDES.

No Drawing. Application filed October 27, 1924, Serial No. 746,248, and in Germany November 14, 1923.

This invention relates to the use of artificial tanning materials in tannery and consists in the valuable discovery that sulfonic acids obtained from lignite tar which is produced by the carbonization of lignite at low temperatures, or from low temperature carbonization tar from other varieties of coal, which products may be comprised by the term "aliphatic tars", or from fractions thereof, have very good tanning properties and may be applied for treating hides or skins either alone or in conjunction with natural or other usual tanning materials. The leather thus obtained has very good properties, especially good body and strength. Tanning may be carried out in the accustomed way employing the sulfonic acids in aqueous solutions of a weak acid character.

The process of tanning according to our invention and the manner of preparing the sulfonic acids afore defined is more fully disclosed by the following examples to which however we do not wish to restrict our invention. The parts are by weight.

## Example 1.

3 parts of a tar oil obtained from lignite (brown coal) tar by fractional distillation and by separating solid paraffin by cooling, is mixed with from 3 to 4 parts of concentrated sulfuric acid of 66 degrees Baumé and the mixture is vigorously stirred at a moderately raised temperature. After a while, the mixture is poured into ice water and the unaltered oil separated from the acid solution, which latter is neutralized with lime, filtered and decomposed with sodium carbonate. It is then ready for tanning which is done in a slightly acidulated and diluted

thick tar and from 5 to 6 parts of monohydric sulfuric acid are vigorously stirred for several hours at a moderately elevated temperature. The sulfonation mixture is worked up as described in Example 1 and the product can be used for tanning in the usual manner employing it in a dilute slightly acid aqueous solution. The product may be used either alone or in mixture with other tanning substances.

What we claim is:

1. The process of tanning which consists in treating hides with a slightly acid solution containing a sulfonation product of an aliphatic tar.
2. The process of tanning which consists in treating hides with a slightly acid solution of a sulfonation product of a fraction of an aliphatic tar.
3. The process of tanning which consists in treating hides with a slightly acid solution containing a sulfonation product of an aliphatic tar and a usual tanning material.
4. As a new tanning composition a slightly acid solution containing a sulfonation product of an aliphatic tar.
5. As a new tanning composition a slightly acid solution containing a sulfonation product of a fraction of an aliphatic tar.
6. As a new tanning composition a slightly acid solution of a sulfonation product of an aliphatic tar and a usual tanning material.
7. As a new tanning composition a slightly acid solution containing a product obtained by the sulfonation of the distillation products of low temperature carbonization tars.

In testimony whereof we have hereunto set our hands.

KURT H. MEYER.  
HERMANN SCHÜTTE.

4 parts of low temperature carbonization